

## UNITED STATES PATENT OFFICE

2,225,100

MANUFACTURE OF SHEETS OR BOARDS  
CONTAINING MINERAL WOOL

Albert L. Clapp, Danvers, Mass.

No Drawing. Application May 9, 1938,  
Serial No. 206,840

10 Claims. (Cl. 92—21)

In my application Serial No. 185,784, filed January 19, 1938, I have disclosed the manufacture of sheets or boards containing mineral wool and more especially long-fibered mineral wool by a process which involves treating or soaking a mass of aggregated mineral or rock wool fibers, as it is available on the market, substantially uniformly with a slimy material and then manipulating the slime-treated or soaked mass in the presence of water, as in a mixing or beater engine, to liberate substantially completely the fibers of the mass and thereby to produce an aqueous suspension of the substantially completely liberated fibers.

The mixing or beater action is controlled to preserve largely or practically completely the original length of the mineral wool fibers in the course of their liberation and suspension in water so that the resulting suspension contains the mineral wool fibers, ranging from a fraction of an inch to several inches, constituting the starting mass of aggregated or tangled mineral wool fibers. Once the aqueous mineral wool fiber suspension is produced, it is possible to spread it substantially uniformly, for instance, to use it much in the same way as plaster for insulating and other purposes, particularly when water-miscible binders, such as sodium silicate, aqueous dispersions of bitumen, resins, or the like, are admixed therewith. In accordance with the aforementioned application, the aqueous mineral wool fiber suspension is produced in a relatively large amount of water, for instance, sufficient water to yield a suspension of about 3% to 4% fiber content, and, after further appropriate dilution with water, is formed into a sheet or board on a paper-making machine.

As described in that application, it is frequently desirable to produce an aqueous suspension of mineral wool fibers blended with cellulose fiber and/or asbestos or the like, in which case, the slime-treated mineral wool fiber mass is added with proper manipulation to an already-prepared aqueous charge of the cellulose fiber and/or to an already-prepared aqueous suspension of the asbestos fiber, as in a beater engine. The resulting aqueous suspension of mineral wool fiber blended with more or less cellulose and/or asbestos fiber is then formed into sheets or boards designed for various purposes, for instance, for use as thermo-insulating material in buildings, refrigerators, and other structures. When the finished sheets are to be used as wallboard or the like, they may contain a substantial proportion of both cellulose and asbestos fiber as well as

mineral wool fiber. However, should the quality of substantial fireproofness be desired in the finished sheets or boards, they may contain little, if any, cellulose fiber and be composed essentially of the mineral wool fiber or a blend of such fiber and asbestos fiber. In some instances, the finished sheets or boards may be impregnated with sizes or binders of various kinds, which, as disclosed in the aforementioned application, may be incorporated into the aqueous fiber suspension from which the sheets or boards are formed and/or be infused into the already-fabricated sheets or boards.

I have now found that when a slimy water-soluble soap solution is used for the purpose of treating or soaking the mass of aggregated mineral wool fibers preparatory to the manipulation of the slime-treated mass in water for the purpose of liberating the individual fibers of which the mass is composed, it is distinctly advantageous that the water in which such manipulation occurs contain a chemical reactive with the water-soluble soap to form a water-insoluble soap gel or slime, for such latter gel or slime is even far more effective than a water-soluble soap slime in promoting the desired loosening and segregation or liberation of the individual fiber units from the mass and thereby yielding the desired aqueous fiber suspension whose fibers are of a length approximating those in the original mass and which is practically devoid of clumps or tangled fibers. It will thus be seen that a slimy water-soluble soap solution is initially used so as to realize the desired penetration and soaking of the mass of aggregated fibers, as this ensures substantially uniform access of the slime to substantially all of the fiber surfaces. Once the fibers in the mass have been substantially uniformly enveloped or protected by the water-soluble soap slime and the mass is to be manipulated in water, it is desirable that the slime resist dispersion or diffusion from the fiber surfaces into the aqueous phase until fiber-liberation has been largely substantially completed; and this is accomplished pursuant to the present invention by converting the water-soluble soap slime on the fiber surfaces to a water-insoluble soap slime through the action of suitable chemicals present in the water, namely, chemicals which furnish the positive radical of a water-insoluble soap, for instance, chemicals of the nature of alkaline earth metal oxide or hydroxide, metal salts, etc. Lime, magnesium oxide or basic carbonate, or equivalent alkaline earth metal compounds are generally preferable by virtue of the fact that they render al-

kaline the aqueous medium in which the slime-treated fiber mass is being manipulated. An alkaline medium evidently functions to preserve the strength of the mineral wool fibers as they are being liberated from the mass and hence minimizes cutting or fracture of the fibers, whereas salts, especially of an acidic nature, such as alum, although useful for the purposes hereof, appear to weaken or "tender" the fibers as they are being liberated and hence to make more difficult the desired preservation of the fibers at substantially their original length.

While not limited thereto, the present invention will now be described in terms of the manufacture of wallboard or insulating board containing asbestos and cellulose fiber. Any suitable cellulose fiber, such as groundwood pulp, and suitable asbestos fiber, preferably short-fibered asbestos, may be added to a beater engine in proportion to yield a finished sheet whose fibrous content will consist of, say, about 25% of asbestos, about 25% of groundwood pulp, and about 50% of the mineral wool fiber. The groundwood pulp not only reduces the cost of the sheet but serves, on account of its short fiber length, to improve its texture or formation. The short-fibered asbestos, which is also inexpensive, not only improves sheet formation but assists to some extent in liberating or individualizing the mineral wool fibers of the slime-treated mineral wool fiber mass subsequently added to the beater engine. The asbestos also enhances the "freeness" of the stock even though it wets up and absorbs water readily. The groundwood pulp and asbestos are mixed in ample water in the beater engine until a substantially uniform aqueous fiber suspension is realized, whereupon about 5% of lime, calculated on all the fibrous components of the finished sheet or board (including the weight of the mineral wool fiber component subsequently added) is admixed with the aqueous suspension of blended asbestos and groundwood pulp.

The mineral wool fiber mass to be added to the fiber suspension in the beater engine is prepared or conditioned for such addition by undergoing a substantially uniform wetting or soaking treatment with an aqueous solution of water-soluble soap in slimy, preferably heated, condition. Specifically, a mass of the aggregated mineral wool fibers consisting of fibers ranging from a fraction of an inch to several inches may be thoroughly soaked with excessive heated soap solution, such as a 3% to 5% solution of sodium stearate or other fatty acid soap. The soap solution may be produced by dissolving the soap in hot water, whereupon, while the soap solution is still hot or warm, the mass of mineral wool may be submersed in an excess of the solution so as to ensure uniform wetting of substantially all the fiber surfaces with the solution. The desired results are had when about 200 parts of the mineral wool fiber mass are plunged into about 1,000 parts of a hot soap solution of about 3% to 5% strength. Excess soap solution may be drained and, if desired, gently squeezed from the mass, but it is preferable that the mass contain upwards of about 150% of its weight of soap solution upon being added to the beater engine.

Upon being added to the beater engine, which contains, for example, a lime water suspension of the asbestos and groundwood pulp, the soap-solution-soaked mass of mineral wool fibers is subjected to manipulation and, in being manipulated, the lime water quickly diffuses to the soapy slime enveloping the fibers and reacts

therewith to form a water-insoluble soap slime, namely, a calcium soap slime. The calcium soap slime resists, on account of its water-insolubility, displacement or dispersion from the mineral wool fiber surfaces. Accordingly, such slime tends to remain present on the fiber surfaces during the manipulation of the aggregated mineral wool fiber mass until the fibers, as a result of the continued manipulation of the mass, have been substantially completely liberated or individualized in the aqueous medium and commingled with the asbestos and groundwood pulp fibers. In other words, the calcium soap slime evidently affords the desired lubricating action on the fibers and is not materially diluted or dispersed in the beater water until the fibers of the mass have substantially completely parted from one another and the originally aggregated fibers of the mass have been resolved into individualized or disaggregated fibers and have been substantially uniformly dispersed along with the asbestos and groundwood pulp fibers in the aqueous medium. The substantially complete liberation and dispersion of the mineral wool fibers in the aqueous medium requires only a comparatively short period of time, for instance, about 5 to 15 minutes or so, the particular time depending, of course, on the particular mixing or beater engine and the amount of stock charged thereto. It might be noted that the mixing or beater engine used for the purposes hereof need not be of that type ordinarily used for papermaking, that is, the type comprising a beater roll equipped with sharp blades or knives arranged in fiber-cutting or beating relationship to a bed-plate. On the contrary, the mixing or beater engine used for the purposes hereof may comprise as its mixing or beating instrumentality nothing more than a paddle wheel, under whose action the desired manipulation or agitation in water of the mineral wool fiber mass is effected in the substantial absence of cutting or fracture of the mineral wool fibers. Indeed, even when the usual beater engine is used for the purposes hereof, its beater roll is raised sufficiently from the bed-plate so that practically all it does is to admix, agitate, or manipulate the mineral wool fiber mass in the beater water. The same sort of manipulation, agitation, or mixing action is also all that is usually necessary for slushing the asbestos and groundwood pulp to form a smooth fiber suspension. The finished aqueous fiber suspension consisting of a blend of mineral wool fiber of substantially original fiber length, asbestos, and groundwood pulp, may be of about 3% stock or fiber content.

Once the mixed substantially completely individualized fiber suspension has been produced in the mixing or beater engine, various sizing agents, fillers, pigments, etc. may be added thereto. For instance, about 5% to 8% cooked or raw starch, based on the dry weight of all the fibrous components, may be added to the fiber suspension so as to enable the realization of a finished sheet or board of marked stiffness by reason of its starch content. Again, alum in the amount of, say, about 2% to 3%, based on the weight of the fibrous components, may be added to the mixed fiber suspension so as to precipitate or fix on the fibers such residual lime and/or water-soluble soap as may have escaped interaction. It is generally preferable, however, to add alum in amount short of imparting an acid condition to the fiber suspension, that is, in amount to leave the suspension at a pH value of, say, 7.5 to 8.5,

for delivery to the papermaking machine. On its way to the papermaking or board-forming machine, the fiber suspension may be diluted with further water to appropriate sheet-forming or board-forming consistency; and, should there be excessive foaming tendency in the suspension on account of its content of calcium fatty-acid soap, suitable anti-foaming agents, such as kerosene and/or paraffin wax emulsion may be added thereto. The sheets and/or boards may be formed on the papermaking machine in much the same way and for much the same purposes as disclosed in my application Serial No. 185,784; and the resulting sheets or boards may, if desired, undergo such after-treatment or after-impregnation with suitable binder, waterproofing material, or the like, as disclosed in that application.

It is to be understood that the process hereof is subject to variation, so far as concerns, for example, such features as the particular water-soluble soap slime used for soaking the mass of mineral wool fiber, the strength of the aqueous water-soluble soap slime, the particular fibrous composition or furnish for the finished sheet or board, and the particular kind of chemical used to convert the water-soluble soap slime in the mineral wool fiber mass to a water-insoluble soap slime as it is being manipulated in water. Generally speaking, it is preferable to use fatty acid soap slimes of the nature of sodium stearate and/or sodium palmitate and/or sodium oleate or the like, but it is possible, of course, to use the potassium soap of the fatty acids or other water-soluble alkali-metal soap solution for initially soaking the mineral wool fiber mass. Although rosin soap slime is not so effective as fatty acid soap slime, yet it may be used in some instances, especially in admixture with fatty acid soap slime. Again, the soap of the substance known commercially as "tallol," which is a by-product of kraft pulp manufacture, may be used. Tallol soap, which may be prepared by saponifying the "tallol" with alkali-metal hydroxide, such as sodium or potassium hydroxide, is a complex material containing fatty acid soap as well as rosin soap; and it may be used as a slimy aqueous solution of suitable strength for soaking the mass of mineral wool fibers. In lieu of forming the sheets or boards hereof from the particular mixed fiber suspension hereinbefore described, that is, a fiber mixture containing about 50% of the mineral wool fibers and about 25% each of asbestos and groundwood pulp, it is possible to form such sheets or boards from an aqueous fiber suspension consisting essentially only of the mineral wool fiber or consisting of a mixture of the mineral wool fiber with, say, about an equal amount of asbestos. Again, it is possible to form the sheets or boards hereof from an aqueous suspension of mixed fibers containing, besides the mineral wool fiber, various proportions of asbestos and cellulose fiber, for instance, chemical wood pulps, such as kraft and/or sulphite pulp, waste papers, rag pulp, etc.; and, if desired, the mixed fiber suspension may contain animal fiber, such as cattle hair, wool, or the like.

It is to be understood that the process hereof constitutes essentially an improvement of the process outlined in my application Serial No. 185,784, more especially in those instances when a water-soluble soap slime is used in initially treating or soaking the mass of mineral wool fiber, and that such improvement consists essentially in converting the water-soluble soap slime into a water-insoluble soap slime by the addition to the

water in which the soaked fiber mass is manipulated of a chemical furnishing the ion (i. e., positive alkaline earth metal or metal ion) combinable with fatty acid to yield water-insoluble fatty acid soap. It is, as already indicated, preferable to disseminate such chemical, e. g., lime, throughout the water in the mixing or beating engine before the addition and manipulation of the soap-solution-soaked mass of mineral wool fiber in the water, but such chemical may be added to the water simultaneously with the addition of such mass or during the very early stages of manipulating such mass in the water. Other than the particular improvement herein indicated, the process hereof is akin to the process of the aforementioned application and may involve the various features indicated in that application.

I claim:

1. A process which comprises treating a mass of aggregated mineral wool fibers with an aqueous slime of water-soluble soap of at least about 3% soap content so as to envelop the fibers substantially uniformly with the slime; and agitating the slime-treated mass of aggregated fibers in water in the presence of a chemical that reacts with said soap and forms a water-insoluble soap slime until the fibers of said mass have been substantially completely liberated to yield an aqueous suspension of the substantially completely liberated fibers. 20

2. A process which comprises thoroughly soaking a mass of aggregated mineral wool fibers with an aqueous slime of water-soluble fatty acid soap of at least about 3% soap content; and agitating such slime-treated mass of aggregated fibers in water containing a chemical that reacts with said soap and forms a water-insoluble soap slime until the fibers of said mass have been substantially completely liberated to yield an aqueous suspension of the substantially completely liberated fibers. 35

3. A process which comprises treating a mass of aggregated mineral wool fibers with aqueous slime of water-soluble soap in amount in excess of that necessary to envelop the fibers substantially uniformly with the slime; removing excess slime from said mass; and agitating said slime-treated mass in lime water, thereby converting said slime into calcium soap slime, until the fibers of said mass have been substantially completely liberated to yield an aqueous suspension of the substantially completely liberated fibers. 45

4. A process which comprises thoroughly soaking a mass of aggregated mineral wool fiber with aqueous slime of water-soluble soap in amount in excess of that necessary to envelop the fiber substantially uniformly; removing excess slime from said mass; and agitating said slime-soaked mass in lime water, thereby converting said slime into calcium soap slime, until the fibers of said mass have been substantially completely liberated to yield an aqueous suspension of the substantially completely liberated fibers, said agitation being controlled to preserve largely the original fiber length of said fibers. 55

5. A process which comprises treating a mass of aggregated mineral wool fibers with aqueous slime of water-soluble soap of at least about 3% soap content in amount in excess of that necessary to envelop the fibers substantially uniformly with the slime; removing excess slime from said mass; adding the slime-treated mass to an already-prepared suspension of asbestos and cellulose fiber in water containing a chemical that reacts with said soap and forms a water-insol- 70

- uble soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.
6. A process which comprises treating a mass of aggregated mineral wool fibers with aqueous slime of water-soluble soap in amount in excess of that necessary to envelop the fibers substantially uniformly with the slime; removing excess slime from said mass; adding the slime-treated mass to an already-prepared suspension of asbestos fiber in water containing a chemical that reacts with said soap and forms a water-insoluble soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.
7. A process which comprises treating a mass of aggregated mineral wool fibers with aqueous slime of water-soluble soap in amount in excess of that necessary to envelop the fibers substantially uniformly with the slime; removing excess slime from said mass; adding the slime-treated mass to an already-prepared suspension of cellulose fiber in water containing a chemical that reacts with said soap and forms a water-insoluble soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.
8. A process which comprises thoroughly soaking a mass of aggregated mineral wool fiber with aqueous slime of at least about 3% concentration of water-soluble fatty acid soap in amount in excess of that necessary to envelop the fiber substantially uniformly; removing excess slime from
- said mass; adding the slime-soaked mass to an already-prepared suspension of asbestos and cellulose fiber in lime water, thereby converting said slime into calcium fatty acid soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.
9. A process which comprises thoroughly soaking a mass of aggregated mineral wool fiber with aqueous slime of water-soluble fatty acid soap in amount in excess of that necessary to envelop the fiber substantially uniformly; removing excess slime from said mass; adding the slime-soaked mass to an already-prepared suspension of asbestos in lime water, thereby converting said slime into calcium fatty acid soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.
10. A process which comprises thoroughly soaking a mass of aggregated mineral wool fiber with aqueous slime of water-soluble fatty acid soap in amount in excess of that necessary to envelop the fiber substantially uniformly; removing excess slime from said mass; adding the slime-soaked mass to an already-prepared suspension of cellulose fiber in water containing lime, thereby converting said slime into calcium fatty acid soap slime; agitating said mass in said water to liberate substantially completely the fibers of said mass and thereby to produce an aqueous suspension of the substantially completely liberated fibers, said agitation being controlled to preserve largely the original fiber length of said mineral wool fibers; and sheeting the mixed fibers from the resulting aqueous suspension.

ALBERT L. CLAPP.